

134  
17  
UNITED STATES PATENT OFFICE.

GOODMAN CHARLES MANDLEBERG, HENRY LESSER ROTHBAND, AND  
SAMUEL LAWRENCE MANDLEBERG, OF MANCHESTER, ENGLAND.

PROCESS OF MANUFACTURING RUBBER GOODS.

SPECIFICATION forming part of Letters Patent No. 441,501, dated November 25, 1890.

Application filed February 5, 1890. Serial No. 339,838. (No specimens.) Patented in England November 14, 1888, No. 16,541; in France March 14, 1889, No. 196,712; in Belgium March 15, 1889, No. 85,405, and in Austria-Hungary August 31, 1889, XXXIX, 1,793 and XXIII, 1,747.

*To all whom it may concern:*

Be it known that we, GOODMAN CHARLES MANDLEBERG, HENRY LESSER ROTHBAND, and SAMUEL LAWRENCE MANDLEBERG, subjects of Her Majesty the Queen of the United Kingdom of Great Britain and Ireland, residing at Manchester, in the county of Lancaster, England, have invented certain new and useful Improvements in the Process of Manufacturing Rubber Goods, (for which we have obtained Letters Patent for the United Kingdom of Great Britain and Ireland, dated November 14, 1888, No. 16,541; in France, dated March 14, 1889, No. 196,712; in Belgium, dated March 15, 1889, No. 85,405, and in Austria-Hungary, dated August 31, 1889, Vol. 39, Fol. 1,793, Vol. 23, Fol. 1,747;) and we do hereby declare the following to be a full, clear, and exact description of the invention, such as will enable others skilled in the art to which it appertains to make and use the same.

The invention relates to the manufacture of water-proof goods and garments, and particularly to rubber goods and garments, and is designed and has for its object important and material improvements whereby such goods or garments are rendered more durable and better adapted for use in warm or hot climates than those heretofore found on the market.

The further object of our invention is to produce odorless rubber goods and garments; and it consists in the process of manufacture, substantially as hereinafter described.

Although our process is applicable to all grades or classes of fabrics heretofore used in the manufacture of these goods, we will describe the same in its application to such goods or garments made from the finer and more delicate single-texture fabrics, and which are more especially designed for wear by ladies.

In carrying out our invention the fabric, whether of cotton, wool, or silk, or a mixture of these fibers, is prepared by what is termed "spreading" or coating in the ordinary way with several coats of the proofing, the first coat of which consists of a "dough" or com-

50 pound of india-rubber, litharge, and a naphtha solvent. The next coat consists of a similar compound, to which is added a vulcanizing agent, such as sulphur. Finally we apply a last coat, substantially like the first, but containing a smaller per cent. of litharge. 55 In practice we usually apply three coats of the compound that contains the vulcanizing agent, and which we term the "intermediate coating," the first and last coating being the foundation or base and the finishing coatings, respectively, one or more of each of which may be applied. We thus obtain a water-proof fabric whose intermediate stratum of waterproofing substance alone contains a vulcanizing agent.

60 The mode of mixing and spreading of the dough, as well as the proportions of the ingredients of the latter, are well known to the trade, and the said proportions of ingredients may be varied, as described or required.

65 In some cases whiting may be added to the dough, or materials equivalent thereto, and when it is desired to produce a "farina finish"—that is to say, when a farina-coated fabric or garment is to be produced—farina or its equivalent is applied in the usual manner. The fabric prepared as described is then partially vulcanized by exposure to a temperature of about 250° Fahrenheit for a 70 short time. This is done in the well-known "stoves," dry air being used as the heating agent. The partially-vulcanized material is then cut up and made into garments in the ordinary manner, the seams being secured together with the usual rubber cement, which is 75 a solution having sulphur in it—that is to say, a cement that will vulcanize. The garments made from the partially-vulcanized material are then completely vulcanized and simultaneously deodorized by exposure to a temperature higher than that used in the partial vulcanization—namely, to a temperature of about 80 260° Fahrenheit. This is also carried out in the usual stoves, and during the earlier part of the stoving process the air laden with the 85 ill-smelling volatile vapors is allowed to escape, this being continued so long as the escaping air is charged with such vapors. A 90 95 152

thoroughly vulcanized and deodorized article is thus obtained.

If desired, the garments may be perfumed by exposure to the vapors or air laden with the vapors of any suitable or desired essential oil—such as oil of lavender, for instance—and this may be effected immediately after the vulcanizing and deodorizing process and in the same apparatus.

10 If the water-proof fabric is intended as a commercial product, the material coated as above described is completely vulcanized and deodorized after the spreading, and perfumed, if desired. The garments made from this material may be subjected to a final stoving process in order to deodorize the cement used for uniting the seams.

The mode of preparing the fabric as described we believe was unknown prior to our 20 invention, and we claim that a more durable and pliable water-proof fabric is thereby obtained. We also believe that before our invention a water-proof garment has not been made from a partially-vulcanized material, 25 whether such material is prepared or coated, as described, or in any other manner, and we claim that by first partially vulcanizing the material, then making the garments and completely vulcanizing the latter, we not only 30 more thoroughly vulcanize the water-proof coatings, but we also more thoroughly deodorize the same and materially enhance the properties of the waterproofing compound and the durability of the garment.

35 Having now described our invention, what we claim, and desire to secure by Letters Patent, is—

1. The process of manufacturing india-rubber garments, substantially as herein described, which consists in partially vulcanizing the proofed or coated fabric, making the garments from such partially-vulcanized fab-

ric, and completely vulcanizing and simultaneously deodorizing the garments.

2. The process of manufacturing india-rubber water-proof fabrics, substantially as herein described, which consists in first coating a fabric with a rubber compound devoid of a vulcanizing agent, next with a rubber compound combined with a vulcanizing agent, 50 and lastly with a rubber compound devoid of a vulcanizing agent, for the purposes specified.

3. The process of manufacturing india-rubber water-proof fabrics, substantially as herein described, which consists in first coating a fabric with a compound composed of rubber and litharge and a suitable solvent; secondly, 55 with a like compound combined with a vulcanizing agent, as sulphur; and, lastly, with a compound similar to that of the first coating 60 but containing less litharge.

4. The process of manufacturing rubber water-proof goods, substantially as herein described, which consists in first coating a fabric with a rubber compound devoid of a vulcanizing agent, then with a rubber compound containing such vulcanizing agent, and lastly with a rubber compound devoid of a vulcanizing agent, exposing the fabric so treated to a temperature of about 250° Fahrenheit to 65 partially vulcanize the same, making the garments from the partially-vulcanized fabric in the usual manner, and subjecting the finished garments to a vulcanizing and deodorizing temperature of about 260° Fahrenheit. 70 75

In testimony whereof we affix our signatures in the presence of two witnesses.

GOODMAN CHARLES MANDLEBERG.  
HENRY LESSER ROTHBAND.  
SAMUEL LAWRENCE MANDLEBERG.

Witnesses:

PETER J. LIRSEY,  
WILLIAM FAULKNER.